

## [54] METHOD FOR CASTING A LARGE LEAD ANODE PLATE

[75] Inventor: Yuki Nishimura, Takehara, Japan

[73] Assignee: Mitsui Mining &amp; Smelting Co., Ltd., Tokyo, Japan

[22] Filed: Feb. 14, 1974

[21] Appl. No.: 442,575

[52] U.S. CL..... 164/128, 164/130, 164/135,  
164/348

[51] Int. Cl..... B22d 25/04, B22d 35/04

[58] Field of Search ..... 164/126, 128, 130, 133,  
164/135, 154, 322-326, 348

## [56] References Cited

## UNITED STATES PATENTS

974,541 11/1910 Truswell ..... 164/326

2,070,821 2/1937 Badger ..... 164/135 X

## FOREIGN PATENTS OR APPLICATIONS

1,006,591 4/1957 Germany ..... 164/126

1,194,103 6/1965 Germany ..... 164/348

Primary Examiner—Robert D. Baldwin

## [57] ABSTRACT

A method is provided for casting a large lead anode plate, which comprises controlling the pouring temperature most favorable to the pumping and pouring of the melt, pouring the melt through a pouring trough into a mold, and applying three stages of water cooling to the resulting casting.

7 Claims, 5 Drawing Figures



PATENTED FEB 4 1975

3,863,703

SHEET 1 OF 2



FIG. 1

PATENTED FEB 4 1975

3,863,703

SHEET 2 OF 2



FIG. 2



(PRIOR ART) FIG. 3



FIG. 4



FIG. 5

# METHOD FOR CASTING A LARGE LEAD ANODE PLATE

## BACKGROUND OF THE INVENTION

Generally, lead anode plates are desirably flat, because the use of flexed lead anode plates in electrolytic cells tends to cause short-circuits and channeling of electric current which decreases the electrolytic efficiency. Heretofore, anode plates for use in lead electrolysis have been prepared by the steps of melting crude lead having a purity of 97.0 to 98.5 percent, pouring the melt into a flat or vertical mold in a thickness of about 30mm, cooling the casting by water, and picking up the resulting casting from the mold. In casting techniques of the prior art, however, the anode plates often have been picked up before they have been sufficiently cooled down. Because the cooling of the casting has not been adequate at the time and speed involved, a flexed anode plate is often produced. The use of such anode plates causes a decrease in electrolytic efficiency and thus it is necessary to press the plate into a flat form before installing the same in an electrolytic cell.

Further, when melted crude lead is pumped from a melting kettle to a mold through a trough or a pipe, the discharge of a large amount of melted lead into a flat mold causes waviness in the mold, resulting in roughness of the surface and/or overflow of the mold causing the casting to swell over the edge of the mold, which phenomenon is referred to as a "picture frame." On the other hand, when the melt is poured in a small amount, there are disadvantages in that casting takes much time and that the melt tends to solidify during the pouring. Therefore, in the prior art the pouring trough was often provided with a screen so that the melt passed a number of notches that were defined in the lower portion of the screen to reduce the adverse effects described above, yet without solving the problem.

Further, in cooling a cast anode plate, either using massive quantities of water or when partial cooling of only one side surface is employed, there is produced a substantial bending stress resulting in flexing of the anode plate, in accordance with cooling methods of the prior art.

## BRIEF SUMMARY OF THE INVENTION

The present invention relates to a method for casting large lead anode plates having a minimum degree of flexion in the resulting product.

More specifically, the method comprises controlling the temperature such that the lowest temperature employed is conducive to proper pumping and pouring of the melt, reducing the velocity of melt without decreasing the volume of flow of melt when pouring melt into a mold, and then applying first and second stages of water cooling to a melt surface followed by a third stage of water cooling to the mold back surface.

For these purposes the pouring temperature employed is within the range of about 340°C to 350°C, and the melt is preferably poured into a mold through a pouring trough provided with two screens, each having a number of circular openings extending over the surface thereof.

The present invention further provides a casting method for producing large lead anode plates in dimensions of 1,150 × 1,000 × (25 – 39)m/m and in weight of 380–440kg during periods of about 12 to 14 sec-

onds. The plates so produced are particularly useful as components in electrolytic cells, such as batteries.

The invention will be more fully understood by reference to the following more detailed description and drawings:

## BRIEF DESCRIPTION OF THE DRAWINGS

FIG. 1 is a schematic drawing illustrating the pouring trough and the anode casting molds of the invention;

FIG. 2 is a histogram illustrating the degree of flexion of lead anode plates of the invention (solid line) in comparison with that of the prior art (dotted line);

FIG. 3 is a schematic drawing illustrating a typical pouring trough of the prior art;

FIG. 4 is a plan view of screen 5 of FIG. 1, illustrating a preferred embodiment of the screen; and

FIG. 5 is an elevational view of a preferred embodiment of screen 3 of FIG. 1.

## DETAILED DESCRIPTION OF THE PREFERRED EMBODIMENT

In the production of large lead anode plates it has been the practice to pour melted crude lead into a suitable mold at a temperature of 365° to 375° C. In view of the fact that lower pouring temperatures are desirable for reducing the bending stress due to cooling and bearing in mind that the melting point of pure lead is 327.3°C, in accordance with the present invention the transportation and pouring of melted crude lead is held and critically controlled within the range of 340° to 350°C, which has been found to be the lowest temperature range at which no difficulty occurs in the pumping and the pouring thereof. Moreover, the handling of the melt is facilitated by two screens in such form as shown in FIGS. 1, 4 and 5, the first positioned at about the midpoint of the trough and the second at about the discharge port of the pouring trough in order to reduce the velocity of the melt without decreasing the volume of flow thereof.

Referring to FIGS. 1 and 5, melted lead flows in the direction of the arrow F in a pouring trough 1 which is provided with a screen 3, at substantially the midway position 2 so that it partially restricts the flow of melted lead, which nevertheless passes through a number of circular openings 3a defined in the screen 3. Trough 1 then changes direction and diverts the flow of melt downwardly and to a discharge port 4 of the pouring trough 1, interrupted at this point by a screen 5 (FIGS. 1 and 4) provided with a number of circular openings 5a defined in the screen 5 which is disposed at the discharge port 4 or at the vicinity thereof. Thereafter, the melted lead is poured into a mold at position P<sub>1</sub>. Thus, it is possible to reduce the velocity of melted lead without decreasing the volume of flow thereof.

In order to maintain the bending stress to the minimum, cooling is effected separately through the melt surface and through the mold surface, and the cooling through the melt surface is divided into first and the second stages, wherein the amount of cooling water is carefully adjusted. The cooling water is preferably at substantially normal room temperature, or below.

FIG. 1 shows a rotatable, cylindrical casting apparatus 6 which comprises 18 mold pieces at the positions P<sub>1</sub> to P<sub>18</sub> representing mold segments which advance in the direction of the arrow R. When, for example, mold P<sub>1</sub> is filled from pouring trough 1 and then the mold is advanced to the position P<sub>5</sub>, the first stage of cooling C<sub>1</sub>

is effected by pouring water onto the mold. When the mold advances to the position  $P_7$ , the second cooling stage  $C_2$  is effected by pouring water onto the mold. While the mold advances from the position  $P_9$  to  $P_{12}$ , the third stage of water cooling is effected by pouring water over the mold surface. Finally, the mold advances to the position  $P_{15}$  where the casting is removed therefrom. The molds are not necessarily limited to 18 pieces, which are shown for illustrative purposes only, since molds having different numbers of pieces can be employed. Further, cooling positions and the removal position of the casting are not limited to the positions in FIG. 1, but may be selected appropriately in accordance with this invention.

The first stage of cooling is preferably conducted with water in an amount of from about 1.0 to 1.5 liters per mold segment. It is preferable that the first cooling be effected at as many points on the surface of a particular mold segment as possible, and more than 10 points are more preferably selected so that the cooling effect can be attained over all of the melt surface. Further, the first stage of cooling is preferably conducted after the lapse of 2 or 3 minutes from the completion of the pouring of the melt.

The second stage of cooling is preferably conducted with water in an amount of 0.5 to 1.0 liter per mold segment and after the lapse of 30 to 60 seconds from the completion of the first stage of cooling. The time duration for application of the cooling water may be about 30 seconds both in the first and second stages of cooling. The third stage of cooling effected through the mold surface is preferably started after the lapse of 30 to 60 seconds from the completion of the second stage of cooling and is conducted by applying water over all of the mold back surface in an amount of 170 liters per minute.

A more specific embodiment of the present invention will be illustrated in comparison with a method according to the prior art. In this case, a casting apparatus having a capacity of producing a large anode plate of  $1,150 \times 1,000 \times (25-39) \text{ m/m}$  and of 380-440 kg in from 12 to 14 seconds is employed.

According to the present invention, a pouring trough 1 illustrated in FIG. 1 is employed, through which melted lead is poured into molds at a pouring temperature of  $340^\circ$  to  $350^\circ\text{C}$ , while water in an amount of 1.0 to 1.5 liter/32 seconds is poured downwardly at 22 points of the melt surface during the first stage of cooling; then water in an amount of 0.5 to 1.0 liter/32 seconds is poured downwardly at 9 points of the melt surface during the second stage of cooling; then water in an amount of 340 liter/2 minutes is poured upwardly over all of the back surface of the mold during the third stage of cooling; and the casting finally removed.

According to a method of the prior art, the pouring trough 11 illustrated in FIG. 3 is employed, through which melted lead is poured into molds at a pouring temperature of  $365^\circ$  to  $375^\circ\text{C}$ , while initially water in an amount of 2.0 to 3.0 liters is poured downwardly at 22 points of a melt surface and then water in an amount of 340 liters is poured upwardly over all of the back surface to provide cooling, before removing the casting.

The frequency distribution of the degree of flection of the anode plates obtained according to the present invention is shown in FIG. 2, in comparison with that of the prior art. It is clear that the anode plates pro-

duced according to the present invention are superior to those of the prior art. Particularly to be noted, the distribution of the preferred embodiment of the present invention (solid line) is clearly defined at a lower flection degree than the distribution in the prior art (dotted line), and the average flection degree (about  $2\text{m/m}$ ) of the preferred embodiment of the present invention is one third smaller than that of the prior art (about  $6\text{m/m}$ ). The deviation in the flection degree of the embodiment of the present invention (about  $\pm 1\text{m/m}$ ) is one second smaller than that of the prior art (about  $\pm 2\text{m/m}$ ), and the maximum value of flection degree of the preferred embodiment of the present invention ( $3\text{m/m}$ ) is much smaller than the minimum flection degree of the example of the prior art ( $5\text{m/m}$ ). Thus, the present invention provides an improved method for producing, with high reliability, an excellent large anode plate having a small flection degree.

Resort may be had to such modifications and equivalents as fall within the spirit of the invention and the scope of the appended claims.

What we claim is:

1. A method for casting a large lead anode plate comprising:

providing at least one open topped anode plate mold; providing a pouring trough opening into said mold; transporting melted crude lead through said trough at a temperature within the range of from about  $340^\circ\text{C}$  to  $350^\circ\text{C}$ ; reducing the velocity of the melt without decreasing the volume of flow of melt during pouring of the melt into said mold; sequentially applying discrete first and second stages of water cooling to the melt surface and a third stage of water cooling to the back surface of the mold; and subsequently removing the cast plate from said mold.

2. A method according to claim 1, comprising pouring said melt into a mold through a pouring trough provided with two screens, one at about the mid position of the trough and the other at about the discharge port thereof.

3. A method according to claim 2 wherein said screens are provided with a number of circular openings extending substantially over the surface thereof.

4. A method according to claim 1, wherein said melt is poured into a mold through a pouring trough provided with two screens, each having a number of circular openings extending substantially over the surface thereof one at about the mid position of the trough and the other at about the discharge port thereof; and cooling water is applied at the rate of about 1.0 to 1.5 liters at more than 10 points on the melt surface for about 30 seconds after the lapse of about 2 to 3 minutes from the completion of pouring of said melt, followed by a second stage of water cooling of the melt surface and a third stage of water cooling applied to the back of the mold.

5. A method according to claim 4, comprising applying water at the rate of about 0.5 to 1.0 liter to a melt surface for about 30 seconds after the lapse of 30 to 60 seconds from the completion of the first stage of water cooling.

6. A method according to claim 4, comprising applying water at the rate of about 170 liters per minute over all of the mold back surface for 2 minutes after completion of the second stage of water cooling.

7. A method according to claim 4, comprising applying water at the rate of about 1.0 to 1.5 liters at 22 points on the melt surface for 32 seconds in the first stage of water cooling, water at about 0.5 to 1.0 liters at 9 points on the melt surface for 32 seconds in the

second stage of water cooling, and water at about 340 liters over all of the mold back surface for 2 minutes in the third stage of water cooling.

\* \* \* \* \*

10

15

20

25

30

35

40

45

50

55

60

65